

1

2,710,839

## ARYL-UREA THICKENED GREASES

Edward A. Swakon, Hammond, and Cecil G. Brannen, Munster, Ind., assignors to Standard Oil Company, Chicago, Ill., a corporation of Indiana

No Drawing. Application November 1, 1952,  
Serial No. 318,321

14 Claims. (Cl. 252—49.6)

The present invention relates to novel lubricant greases and to the method of preparing same. More particularly, it relates to novel greases comprising a lubricant vehicle thickened with certain high melting aromatic ureido and amido compounds. Greases of this type, particularly those wherein the lubricant vehicle comprises a silicone polymer oil, have demonstrated exceptional stability and lubricity at elevated temperatures.

As lubricants are required to perform at higher and higher temperatures because of increased speeds of engines and machines, the advent of jet propulsion, atomic energy as a source of power, etc., it has become increasingly difficult to prepare greases fulfilling the requirements of such lubricants. In attempting to provide such greases, the art has progressed from the use of petroleum lubricant vehicles thickened with metal soaps of long chain fatty acids, e. g. lithium hydroxystearate, to more thermally stable synthetic lubricating oils such as the aliphatic diesters of dicarboxylic acids, silicone polymers, etc., thickened with such soaps or inorganic materials such as silica gels. The progress of thickener research has not in general, however, kept pace with the development of lubricant vehicles. And at temperatures as high as 400° to 450° F. there are few if any greases available which will retain their consistency and lubricity for any substantial period of time.

In recent years various synthetic lubricant vehicles, e. g. the silicones, fluorocarbons, etc., have been found to be potentially valuable for use in greases employed at very high temperatures because of their thermal stability and relatively low volatility. Unless, however, a thickener having substantially the same degree of thermal stability is available to produce a grease from such an oil, they are of little use. It has now been found that certain very high melting aromatic ureas, di-ureas, amides, and di-amides, all of which contain at least one



radical, wherein R is an aryl radical, and which may hereinafter be referred to broadly as arylcarbamyl compounds, may be employed to thicken silicone polymer oils, as well as other known lubricant vehicles, to produce greases which are stable and display excellent lubricant properties at high temperatures. Whereas silicone polymer oils are particularly preferred for use in greases employed at temperatures as high as about 450° F., other lubricant vehicles, either natural or synthetic, may also be thickened with these materials to produce greases of particular utility between about 250° F. and about 400° F.

It is a primary object of the present invention to provide lubricant greases which are stable and give excellent lubrication at elevated temperatures. A further object is to provide a readily producible series of greases embodying a novel class of thickening agents capable of yielding lubricants particularly suitable for use at temperatures of from about 250° F. to about 450° F. A

2

particular object of the present invention is to provide greases which are effective lubricants at temperatures as high as about 450° F. for substantial periods of time. These and additional objects will be apparent from the following detailed description.

We have found that lubricating vehicles such as silicone polymer oils, mineral lubricating oils derived from petroleum, synthetic lubricating oils such as polyalkylene glycols and their derivatives, high molecular weight esters of dicarboxylic acids, etc. and preferably the silicone polymer oils may be thickened to grease consistency by the addition thereto of from 5 to 70% and preferably from about 10 to about 50% of an arylcarbamyl compound selected from the group consisting of aromatic ureas, di-ureas, amides, and di-amides. Thus, in accordance herewith, arylcarbamyl compounds having the following empirical structure are contemplated as thickening agents in the art of grease manufacture:



In the above formulae, R, R' and R'' represent aryl or alkyl aryl radicals. With the exception that R'' is necessarily a divalent radical, e. g. phenylene, biphenylene, naphthylene, etc., these radicals may be the same or different, e. g. phenyl, biphenyl, naphthyl, etc. in each compound. The aryl or alkyl aryl radicals may be substituted radicals containing various reactive substituents such as hydroxy, carboxy, halo, nitro-, etc.

Examples of amides and di-amides which have been found to yield excellent greases when employed as thickeners are N-benzoyl-4-aminobiphenyl, N,N'-dibenzoyl-benzidine, N,N'-dibenzoyl-p-phenylene-diamine and N,N'-bis-(p-nitrobenzoyl)-benzidine. Such compounds may be readily prepared by techniques well known to the art, e. g. by reaction of an aromatic amine or diamine such as phenylene-diamine, aniline, benzidine, etc., with an aryl halide, e. g. benzoyl chloride. Diamides such as 50 may be prepared by reacting an aromatic monoamine, e. g. aniline, with an aryl halide such as a phthalyl chloride, may likewise be employed in accordance herewith. These compounds may be employed alone or in combination to thicken oleaginous vehicles to grease consistency.

Examples of various ureas and di-ureas which have been found useful as thickeners in accordance herewith are p-carboxy-1,3-diphenylurea; p-chloro-1,3-diphenylurea; 1,3-di-(1-naphthyl)-urea; 4,4'-bis-[3-(p-biphenyl)-ureido]-biphenyl; 1-(p-carboxyphenyl)-3-(p-biphenyl)-urea; 1-(p-carboxyphenyl)-3-(o-biphenyl)-urea; 1,3-di-(p-biphenyl)-urea; 1,3-di-(o-biphenyl)-urea; 4,4'-bis-(3-phenylureido)-3,3'-dimethoxy biphenyl; p-phenylurethan-1,3-diphenyl-urea; p-cyano-1,3-diphenyl-urea; 1-(2,5-dichlorophenyl)-3-phenyl-urea; 4,4'-bis-[3-(2,5-dichlorophenyl)-ureido]-biphenyl; 1,4 - bis-[3-(2-chlorophenyl)-ureido]-benzene; 1,4 - bis - [3-(3-chlorophenyl)-ureido]-benzene; 1,3 - bis - [3-(3-chlorophenyl)-ureido]-benzene, and 1,3-bis-[3-(2-chlorophenyl)-ureido]-benzene. Compounds of this type may readily be prepared by reacting an amine or diamine such as aniline, benzidine, phenylene-

diamine, etc. with an isocyanate of benzene, diphenyl, etc. It should be understood that the specific aryl carbamyl compounds set forth above are enumerated for purposes of illustration and not of limitation. Compounds of this class may be employed alone or in combination with other such compounds to thicken oleaginous vehicles in accordance herewith.

Greases prepared with thickeners of the type described above, particularly those prepared from silicone oil, are exceptionally stable at elevated temperatures with those prepared from ureido compounds being slightly superior to those prepared from amido type thickeners.

The silicone polymer oils which may be employed in accordance with the present invention are those falling substantially within the lubricating oil viscosity range. In general, such oils have the following unit structure:



wherein R and R' represent substituted or unsubstituted alkyl, aryl, alkylaryl, arylalkyl or cycloalkyl radicals. Such compounds may be produced by well-known methods, e. g. the hydrolysis of dialkyldichlorosilanes or dialkyldiothoxysilanes with a suitable chain stopper, e. g. a tri-substituted mono-chlorosilane. For purposes of the present invention, those polymers which are high boiling liquids within the lubricating oil viscosity range are suitable, these generally possessing a viscosity at 100° F. which is within the range of from about 25 to about 3500 S. S. U. It is preferred, for purposes hereof, to employ such oils as have a viscosity at 100° F. of from about 300 S. S. U. to about 1250 S. S. U. Such products are generally colorless and inert, have a very low volatility and undergo relatively slight change in viscosity for a given change in temperature. Relatively common oils of this type are dimethylsilicone polymer, phenylmethylsilicone polymer, chlorophenylmethylsilicone polymer, etc., it being preferred to employ the phenylmethylsilicone polymer in accordance herewith. Methods of preparing such compounds are taught in numerous patents, e. g. U. S. 2,410,346, U. S. 2,456,496, and in the literature such as "Chemistry of the Silicones" by Rochow, page 61, et seq. A particularly desirable phenylmethylsilicone polymer for use in accordance with the present invention is Dow-Corning 550 silicone fluid, a product of Dow-Corning, Inc., which has a viscosity at 100° F. of about 300 to about 400 S. S. U.

Other oleaginous vehicles which may be employed herewith are, for example, mineral oils in the lubricating oil viscosity range, i. e. from about 80 S. S. U. at 100° F. to about 300 S. S. U. at 210° F. These mineral oils are preferably solvent extracted, to substantially remove the low V. I. constituents, e. g. aromatics, with phenol, furfural, B,B'-dichlorodiethylether (Chlorex), liquid SO<sub>2</sub>, nitrobenzene, etc. Synthetic lubricating oils resulting from polymerization of unsaturated hydrocarbons or other oleaginous materials within the lubricating oil viscosity range such as high molecular weight polyoxyalkylene compounds such as polyalkylene glycols and esters thereof, aliphatic diesters of dicarboxylic acids such as the butyl, hexyl, 2-ethylhexyl, decyl, lauryl, etc. esters of sebacic acid, adipic acid, azeleic acid, etc., may be thickened by the aryl carbamyl compounds of the present invention to produce excellent greases. Polyfluoro derivatives of organic compounds, particularly hydrocarbons, in the lubricating oil viscosity range have shown excellent promise when thickened with compounds of the present invention.

Greases of the present invention may be produced by one of the following methods:

(1) The thickener may be prepared apart from and then admixed with the lubricant vehicle and milled in a colloid mill, 3-roll mill, etc.

(2) The thickener may be formed in situ in the oil by introducing the reactants and the desired amount of lubricant vehicle, heating to about 450° F. for a relatively short time, e. g. from about five minutes to an hour to drive off volatile by-products, and then cooling and milling the mixture.

(3) As a slight modification of method 2 above, a solvent such as dioxane may be employed as a diluent and mutual solvent for the reactants. The solvent is then evaporated and the grease is milled, etc. substantially as set forth.

(4) As a step in any of the above three methods, it has been found, when employing a silicone vehicle, that improved properties may be imparted to the grease by "heat-treating" the grease mixture, i. e. subjecting same to a temperature of about 450° F. for at least about half an hour and preferably longer, e. g. from about 1 to 20 hours. Prolonged heating at such temperature may evaporate a portion of the lubricant vehicle; this loss should be replaced and then the mixture should be milled. If desired, the heating and readdition of vehicle may be repeated before milling.

Table 1

| Thickener                                                  | Class                                                          | Percent<br>(By Wt.) | Method of<br>Prepara-<br>tion | Hours Be-<br>fore Failure<br>in Bearing<br>Test | Remarks                                                              |
|------------------------------------------------------------|----------------------------------------------------------------|---------------------|-------------------------------|-------------------------------------------------|----------------------------------------------------------------------|
| N-Benzoyl-p-aminobenzoic acid-----                         | $\begin{array}{c} O \\    \\ RCNHR' \end{array}$               | 33                  | (3) (4)                       | 337                                             | #1 or #2 grade* grease of excellent texture.                         |
| N,N'-Dibenzoylbenzidine-----                               | $\begin{array}{c} O \\    \\ RCNHR''NHCOR \\ O \end{array}$    | 26                  | (2) (4)                       | 188                                             | Smooth #1 grade* grease—very low evaporational loss and low leakage. |
| 4,4'-bis(3-biphenylureido)-biphenyl-----                   | $\begin{array}{c} O \\    \\ RNHCNHR''NHCNHR \\ O \end{array}$ | 20                  | (3) (4)                       | 437                                             | Good appearing #2 grade* grease—highly stable.                       |
| Do-----                                                    | $\begin{array}{c} O \\    \\ RNHCNHR''NHCNHR \\ O \end{array}$ | 18                  | (3) (4)                       | 448                                             | Do.                                                                  |
| 4,4'-bis[3-(2,5-dichlorophenyl)-ureido] bi-<br>phenyl----- | $\begin{array}{c} O \\    \\ RNHCNHR''NHCNHR \\ O \end{array}$ | 25                  | (3) (4)                       | 436                                             | Smooth buttery #1 or #2 grade* grease.                               |
| p-carboxy-1,3-diphenylurea-----                            | $\begin{array}{c} O \\    \\ RNHCNHR' \end{array}$             | 29                  | (3) (4)                       | 653                                             | Good appearance—#2 grade* grease.                                    |
| Do-----                                                    | $\begin{array}{c} O \\    \\ RNHCNHR' \end{array}$             | 23                  | (3) (4)                       | 446                                             | Do.                                                                  |
| 4,4'-bis(3-p-tolylureido)-biphenyl-----                    | $\begin{array}{c} O \\    \\ RNHCNHR''NHCNHR \\ O \end{array}$ | 20                  | (3) (4)                       | 481                                             | Smooth buttery #2 grease.                                            |

\*N. L. G. I. consistency grades.

The method of forming the thickener in situ in the lubricant vehicle described above is claimed in our co-pending Serial No. 392,996 filed November 18, 1953.

In Table 1 are set forth the data obtained on certain greases comprising DC 550 (phenylmethyl silicone polymer oil product of Dow Corning, Inc. having a methyl-phenyl ratio of about 0.6 and viscosity of about 300 to 400 S. S. U. at 100° F.) thickened in accordance herewith. The bearing test referred to in the table is a tentative one adopted by the Coordinating Research Council during the last war and is generally referred to as the A. B. E. C.-N. L. G. I. Test. It is conducted as follows:

3 grams of grease are placed in each of two bearings disposed on the test spindle. One bearing, a special heat treated precision 204 Norma-Hoffman bearing, is subjected to a temperature of 450° F. in an oven, the other bearing, a standard New Departure 204 bearing, is at room temperature. Temperature is determined by a thermocouple inserted in the grease between the races of the bearing in the oven. Failure is adjudged to occur when (1) the temperature in the test bearing reaches 470° F. or higher, (2) wattage in excess of 300% of normal wattage as required, or (3) the bearing does not turn over at the beginning of a test cycle (the test is conducted in cycles of 20 hours operating and 4 hours at rest).

In Tables 2 and 3, below, are set forth data on greases comprising lubricant vehicles other than silicone oil thickened with p-carboxyl-1,3-diphenyl-urea and 4,4'-bis-(3-phenylureido)-biphenyl, respectively.

Table 2

| Lubricant Vehicle                    | Percent (By Wt.) of Thickener | Consistency <sup>1</sup> (Kaufmann Micropenetration) | Method of Prep. |
|--------------------------------------|-------------------------------|------------------------------------------------------|-----------------|
| Ucon 818 <sup>2</sup>                | 33                            | 104                                                  | (1)             |
| Di-2-ethylhexylsebacate <sup>2</sup> | 40                            | 163                                                  | (3)             |
| Tricresyl phosphate                  | 41.5                          | 143-145                                              | (3)             |

<sup>1</sup>  $C_7H_{15}COOCH_2(CH_2OCH_2)_xCH_2OCOC_7H_{15}$  where  $x$  is such as to result in a material within the lubricating oil viscosity range.

<sup>2</sup> The composition of this vehicle was as follows: 90.6% di-2-ethylhexyl sebacate, 3.9% commercial acrylic base V. I. improver, 5.0% tricresyl phosphate, 0.001 U of silicone anti-foam, and 0.5% phenothiazine.

<sup>3</sup> Kaufmann micropenetration.

Table 3

| Lubricant Vehicle                   | Percent (By Wt.) of Thickener | Consistency <sup>1</sup> | Method of Prep. |
|-------------------------------------|-------------------------------|--------------------------|-----------------|
| Benzyl benzoate                     | 30                            | 54                       | (3)             |
| A. T. F. Extracted Oil <sup>2</sup> | 25                            | 47                       | (3)             |
| Fluorocarbon Oil <sup>3</sup>       | 12                            | 95                       | (3)             |

<sup>1</sup> Kaufmann micropenetration.

<sup>2</sup> Petroleum oil of high aromatic content.

<sup>3</sup> Kel-F Polymer No. 40 (product of The M. W. Kellogg Co.).

Greases of the type set forth in the above tables are stable at high temperatures although generally somewhat less stable than those prepared with silicone oil as the lubricant vehicle. Accordingly, they are more suitably employed at temperatures in the range of from about 250° F. to about 400° F. It should be understood, in any event, that while the greases of the present invention are particularly suitable for use at temperatures above 250° F. they are also extremely useful at lower temperatures. Surprisingly, greases of this type, e. g. a silicone thickened with p-carboxy-1,3-diphenyl urea, having exhibited exceptional properties at extremely low temperatures. Thus, as indicated in the following table, a grease comprising D. C. 550 silicone oil thickened with 25% by weight of p-carboxy-1,3-diphenyl urea (Grease A) exhibits substantially better low temperature properties than a grease comprising D. C. 550 thickened with 20% by weight of lithium-12-hydroxy stearate (Grease B). It will be noted that of the two greases the grease of the present

invention, although possessing the greater consistency at room temperature, exhibits greater fluidity at sub-zero temperatures.

Table 4

| Shear Rate (sec <sup>-1</sup> ) | Apparent Viscosity Data <sup>1</sup> |         | Low Temperature Torque <sup>2</sup> (-40° F. under 2,000 gm.-cm. load) | Penetration <sup>3</sup> (Worked) |  |  |
|---------------------------------|--------------------------------------|---------|------------------------------------------------------------------------|-----------------------------------|--|--|
|                                 | Apparent Viscosity (poises)          |         |                                                                        |                                   |  |  |
|                                 | Temperature                          |         |                                                                        |                                   |  |  |
|                                 | -40° F.                              | -65° F. |                                                                        |                                   |  |  |
| Grease A                        | 15                                   | 6,269   | 43,740                                                                 | Seconds 13.5 291                  |  |  |
|                                 | 24                                   | 5,593   | 30,750                                                                 |                                   |  |  |
|                                 | 39                                   | 4,924   | 21,250                                                                 |                                   |  |  |
| Grease B                        | 15                                   | 12,100  | <60,000                                                                | 19.5 330                          |  |  |
|                                 | 24                                   | 10,080  |                                                                        |                                   |  |  |
|                                 | 39                                   | 7,680   |                                                                        |                                   |  |  |

<sup>1</sup> Method and apparatus are described in ASTM Standards on Petroleum Products and Lubricants Method D1092-51.

<sup>2</sup> See Specification MIL G-3278 25 August 1950.

<sup>3</sup> Same reference at (1) above, method D217-48.

As is well known the lithium 12-hydroxy stearate greases exhibit lower apparent viscosities at any given shear rate than other metal base soaps, e. g. calcium, sodium, etc. The data in the above table clearly indicate that the urea thickened grease may be employed at even lower temperatures than the lithium soap grease. These greases may have added thereto antioxidants, oiliness agents, extreme pressure additives, etc. without in any way departing from the scope of the present invention.

Having thus described our invention, what we claim as novel and desire to protect by Letters Patent is defined by the following claims:

1. A lubricant grease comprising a lubricant vehicle thickened with from 5 to 70% by weight of at least one aryl-carbamyl compound melting above about 250° F. which compound is selected from the group consisting of



55 wherein R and R' represent hydrocarbon radicals containing no more than 12 cyclic carbon atoms, which radicals are selected from the group consisting of aryl, alkyl aryl, substituted aryl, and substituted alkyl aryl radicals, and R'' represents a divalent hydrocarbon radical containing no more than 12 cyclic carbon atoms, which radical is selected from the group consisting of arylene, alkyl arylene, substituted arylene, and substituted alkyl arylene radicals.

2. The lubricant grease of claim 1 wherein the lubricant vehicle comprises a silicone polymer oil in the lubricating viscosity range.

3. The lubricant grease of claim 1 wherein the lubricant vehicle comprises an acyclic ester of an aliphatic dicarboxylic acid in the lubricating oil viscosity range.

4. The lubricant grease of claim 1 wherein the lubricant vehicle comprises a polyoxalkylene compound in the lubricating oil viscosity range.

5. The lubricant grease of claim 1 wherein the lubricant vehicle comprises a mineral lubricating oil derived from petroleum.

6. The lubricant grease of claim 1 wherein the lubricant vehicle comprises a polyfluoro-compound in the lubricating oil viscosity range.

7. A lubricant grease comprising a lubricant vehicle thickened with from 5 to 70% by weight of at least one aryl carbamyl compound melting above about 400° F. which compound is selected from the group consisting of



and

10

15

20

ened with from about 5 to 70% by weight of 4,4'-bis-[3-(2,5-dichlorophenyl)-ureido]-biphenyl.

13. The method of preparing a lubricant grease which comprises milling a mixture comprising essentially a lubricant vehicle and from about 5% to about 70% by weight of an aryl carbamyl compound melting above about 250° F. selected from the group consisting of



wherein R and R' represent hydrocarbon radicals containing no more than 12 cyclic carbon atoms, which radicals are selected from the group consisting of aryl, alkyl aryl, substituted aryl, and substituted alkyl aryl radicals, and R'' represents a divalent hydrocarbon radical containing no more than 12 cyclic carbon atoms, which radical is selected from the group consisting of arylene, alkyl arylene, substituted arylene, and substituted alkyl arylene radicals.

14. The method of claim 13 wherein the lubricant vehicle is a silicone oil in the lubricating oil range and said silicone oil and said aryl carbamyl compound are heated to a temperature between about 400° F. and 450° F. for a period of from about 1/2 an hour to about 20 hours prior to milling said mixture.

#### References Cited in the file of this patent

#### UNITED STATES PATENTS

|           |                    |               |
|-----------|--------------------|---------------|
| 2,041,733 | Werntz             | May 26, 1936  |
| 2,070,991 | Hund et al.        | Feb. 16, 1937 |
| 2,468,534 | Young et al.       | Apr. 26, 1949 |
| 2,547,728 | Abrams             | Apr. 3, 1951  |
| 2,550,746 | Wohnsiedler et al. | May 1, 1951   |
| 2,594,286 | Bryant et al.      | Apr. 29, 1952 |
| 2,604,449 | Bryant et al.      | July 22, 1952 |

wherein R and R' represent hydrocarbon radicals containing no more than 12 cyclic carbon atoms, which radicals are selected from the group consisting of aryl, alkyl aryl, substituted aryl, and substituted alkyl aryl radicals, and R'' represents a divalent hydrocarbon radical containing no more than 12 cyclic carbon atoms, which radical is selected from the group consisting of arylene, alkyl arylene, substituted arylene, and substituted alkyl arylene radicals.

8. A lubricant grease comprising essentially a silicone polymer oil in the lubricating oil viscosity range thickened with from about 5 to about 70% by weight of p-carboxy-1,3-diphenylurea.

9. A lubricant grease comprising essentially a silicone polymer oil in the lubricating oil viscosity range thickened with from about 5 to about 70% by weight of N-benzoyl-p-aminobenzoic acid.

10. A lubricant grease comprising essentially a silicone polymer oil in the lubricating oil viscosity range thickened with from about 5 to 70% by weight of N,N'-dibenzoyl-benzidine.

11. A lubricant grease comprising essentially a silicone polymer oil in the lubricating oil viscosity range thickened with from about 5 to 70% by weight of 4,4'-bis-[3-(p-biphenyl)-ureido]-biphenyl.

12. A lubricant grease comprising essentially a silicone polymer oil in the lubricating oil viscosity range thick-

40

45